

# UNITED STATES PATENT OFFICE.

AUGUST LEUCHTER, OF BROOKLYN, NEW YORK.

## ELECTROLYTIC PRODUCTION OF PRINTING-PLATES AND THE LIKE.

1,003,187.

Specification of Letters Patent. Patented Sept. 12, 1911.

No Drawing.

Application filed April 23, 1909. Serial No. 491,727.

To all whom it may concern:

Be it known that I, AUGUST LEUCHTER, a citizen of the United States, and a resident of Brooklyn, in the county of Kings and 5 State of New York, have invented certain new and useful Improvements in the Electrolytic Production of Printing-Plates and the Like, of which the following is a specification.

10 The invention relates to a novel method of producing a new printing surface or plate and the like.

It is well known that electrotypes and analogous printing blocks and plates are 15 commonly made of copper and that the softness of the printing surfaces has occasioned so much loss and annoyance that various processes have been resorted to with the view of producing improved and more durable 20 printing surfaces. These prior processes have not, as is commonly known, produced entirely satisfactory results. In some of them hard printing surfaces have been produced but they have been too thin and 25 also too brittle to be considered entirely efficient or adaptable for general use, especially on modern high-speed cylinder presses. Notwithstanding the various endeavors made to improve electrotype printing plates, the copper 30 per plates are generally in use. A copper printing plate possesses many good qualities, owing to its ease of production, lack of brittleness and other characteristics, but the copper plate lacks durability and the capability of 35 withstanding the heavy modern press-pressures, as well as the capacity of faithfully portraying color or delicate lights and shades to the degree desired in reproductions of fine half-tone plates. One attempt 40 to improve the copper plates and especially to render them more durable, has been by depositing, in an electrolytic bath, a thin film of nickel over the finished copper plate. This film of nickel was necessarily so 45 thin as to add little increased life to the plate and in addition deprived the plate of a portion of the sharpness of delineation it would otherwise have possessed. Another attempt to improve printing plates has been 50 by depositing nickel to form a very thin shell over the surface of the wax mold or case and then depositing copper on and as a backing for said shell. One difficulty connected with this latter process is that nickel

sulfate alone will not only not deposit readily but will not travel over the entire surface of the wax mold or case to produce the shell, and the result has been that in carrying out the process it has been deemed necessary to use a double salt in the bath, whereby 55 a complete though less durable shell has ensued, or to deposit a thin film of another metal over the graphite-treated face of the wax mold or case and then deposit the nickel on this film. The result of this, however, is 60 that the plate has a comparatively soft face, when a hard one is desired. A thick nickel shell can not be successfully produced on a wax surface treated only with graphite, 65 since it will split open during its attempted 70 formation.

The object accomplished by my invention is the production, in an electrolytic bath, of a printing surface of requisite or any desired thickness possessing the characteristics of 75 durability, hardness and lack of brittleness. This printing surface may be formed of any thickness but for the sake of economy in materials, speed of production and general requisites in practical commercial practice 80 will generally be deposited in the form of a shell on the wax mold or case and backed by a deposit of copper.

The printing surface produced in accordance with my invention is harder than either 85 nickel or iron and possesses great tensile strength; it has the hardness of steel and lacks brittleness; it can be readily removed from the wax mold or case; it faithfully reproduces the finest delineations of the mold; 90 it is non-corrosive under all the conditions that printing plates are usually subjected to; it is extremely durable, and its cost of production is not greatly in excess of that of a copper printing surface while it is far 95 more durable and more economical of use.

In carrying out my invention I prepare the wax case or mold in the customary manner up to and including the step of black-leading and washing off of the same, and 100 hence this portion of the general process, being commonly known and practiced by electrotypers, need not be specifically described.

My process involves the production in an electrolytic bath, of the printing surface on 105 and in reproduction of the delineations presented by the face of the wax case or such mold as may be used, and said surface is

formed by depositing in one continuous operation iron and nickel on the mold to produce a plate or shell, which may thereafter be backed, if desired, by a deposit of copper or other metal. The printing surface, whether a plate or a shell, is thus formed of a composite metal or alloy and is therefore neither a nickel or an iron surface but a surface of peculiar nature and possessing characteristics not present in, so far as I am aware, any printing surface heretofore known.

In the practice of my process I preferably employ the nickel as the anode and an iron salt, preferably sulfate of iron, in the bath, and the mold having been hung in the bath in the customary manner as a cathode, the deposition of the iron and nickel on the mold will follow. In the production of electro-  
20 types, the action of the bath will be permitted to continue until a shell of the requisite thickness has been formed, and thereafter the mold and shell will be removed from the bath and submitted to another electro-  
25 lytic bath in which a copper backing will be deposited on the shell. By my process I am enabled to successfully make the plate or shell of any desired thickness in the nickel-  
and-iron bath, but for the sake of economy  
30 in producing electrotypes I prefer to form the plate or shell of only the requisite thickness and then back it up with copper, which is cheaper than the metal of the shell. In carrying on the process and in the continuous use of the main bath, I add iron salt  
35 to the bath from time to time, as shown to be necessary by a hydrometer, so as to maintain the strength or specific gravity of the solution.

40 While I prefer to employ the nickel as an anode and the iron in the bath, I desire it understood that my invention also comprises the use of iron as the anode and nickel in the bath.

45 The printing plate produced in accordance with and embodying my invention possesses hardness to an exceptional degree coupled with tensile strength and springiness, and it may be bent into curved form for cylinder presses without any previous annealing. The strength of my plate is such  
50 that it may be made of considerable thinness and yet possess a durability enabling it to do the work of four or five successive copper plates without change in its printing face.

55 My invention is of particular value in the production of electrotype plates, since the deposited shell however thin it may be, may owing to its tensile strength and flexibility, be readily stripped from the wax surface. A shell of iron would require, owing to its brittleness, to be formed of considerable thickness, as compared with the shell of my invention, and would become distorted un-

der the heat used in the "backing-up" step or the securing of the plate to the type-metal, as commonly practiced.

The fact that my printing plate possesses the characteristics of hardness and springiness or flexibility, is of very great advantage and adapts it for efficient use on modern high speed cylinder presses.

The advantages of securing a hard printing surface of uniform character and proper thickness are obvious and such surface is produced by my invention. In addition the plate made in accordance with my invention faithfully reproduces the finest delineations of the wax case or mold and hence is well adapted for the reproduction of half-tone plates of the highest character. One reason why my plate so faithfully reproduces the finest delineations of the wax surface is that the nickel and iron together will deposit perfectly on the black-leaded wax surface and that the customary metallization of the wax surface by means of a film of copper or silver or the like thereon is entirely avoided, and which metallization step when employed naturally produces an outer surface on the plate which is more or less soft and not capable of withstanding heavy pressure or portraying the delicate color required in half-tone work.

95 The printing surface produced by my invention and composed of nickel and iron in one homogeneous composite layer or thickness differs essentially from a nickel surface or an iron surface or a nickel surface on an iron surface or an iron surface on a nickel surface or a plate made up of a layer of one metal superimposed on a layer of a different metal.

100 The plate of my invention while initially costing more than a copper plate is capable of ready production at reasonable expense and at less expense than a nickel surface, although superior thereto since the nickel for the anode may be purchased at present prices for about fifty cents per pound and the iron sulfate for three and one-half cents per pound. In practical use the plate of my invention will outlast several copper plates and hence is more economical of use than copper plates.

110 I have discovered not only that the nickel and iron produce a printing surface of exceptional merit but that in carrying out my process the nickel and iron readily deposit and work together harmoniously, whereby a surface of uniform character is secured.

115 One economy secured in the use of my plates above copper and other heretofore known plates is that they are capable when set up with other matter on a press, of withstanding long runs without change in their printing face, whereas under like conditions copper plates will have to be removed and renewed from time to time, rendering nec- 125

essary the stopping of the press and the "making ready" of the form, which in itself is a matter greatly to be avoided.

I not only attain economy in the practice 5 of my invention but secure a printing plate which in itself is characteristically different from the plates of the prior art.

I have described my invention as embodied in a printing plate for use in a printing 10 press but do not confine my invention exclusively to a printing plate in a strictly technical sense, since the plates produced by my invention may be employed for stamping and embossing and in other ways 15 for reproducing the designs delineated on them. My invention is of special utility however for use in printing presses and particularly in modern high-speed presses used for long runs.

20 What I claim as my invention and desire to secure by Letters-Patent, is:

1. The process of producing a printing plate in an electrolytic bath which consists 25 in preparing a mold bearing the characters to be produced in the plate, metallizing the surface thereof, suspending the same in the bath, simultaneously depositing nickel and iron electrolytically as an alloy on said metallized surface, to form the plate, 30 removing the mold and plate from the bath, and then depositing in another bath a different metal on the back of the plate to form a backing therefor.

2. The process of producing a printing 35 plate in an electrolytic bath which consists in preparing a mold bearing the characters to be produced in the plate, metallizing the surface thereof, suspending the same in the bath, simultaneously depositing nickel and iron electrolytically as an alloy on said metallized surface to form the plate, with

the nickel as the anode and the iron salt in the solution; removing the plate from the mold, and backing the plate.

3. The process of producing a printing 45 plate in an electrolytic bath which consists in preparing a mold bearing the characters to be produced in the plate, metallizing the surface thereof, suspending the same in the bath, simultaneously depositing nickel and iron electrolytically as an alloy on said metallized surface to form the plate, with the nickel as the anode and the iron salt in the solution, removing the mold and plate from the bath, and then depositing in another bath a different metal on the back of the plate to form a backing therefor.

4. The process of producing electrolytically a plate in reproduction of the surface of a mold, which consists in preparing the 60 mold in wax, metallizing the surface thereof by a black-leading method, suspending the mold in the bath, simultaneously depositing nickel and iron electrolytically as an alloy on said metallized surface to form the plate, 65 removing the mold and plate from the bath, and backing the plate, the nickel in such process being in the form of an anode suspended in the bath and the iron a salt in solution in the bath.

5. The method of making an electrotype comprising electrolytically depositing upon the conducting surface of a mold an alloy of nickel and iron, and applying a backing of another metal to said deposited alloy.

Signed at New York city, in the county of New York and State of New York, this 22nd day of April A. D. 1909.

AUGUST LEUCHTER.

Witnesses:

CHAS. C. GILL,  
ARTHUR MARION.